

Hayward & Lees.

Pile for Making Railroad Rails.

N<sup>o</sup> 49,904.

Patented Jul. 14, 1868.

Fig. 2



Fig. 1



Witnesses.

Wm A Morgan

G. Le. Leotton

Inventor

W. Haywood

J. Lees

per Murphy

Attorneys

# UNITED STATES PATENT OFFICE.

WILLIAM HAYWARD AND JOHN LEES, OF DANVILLE, PENNSYLVANIA.

## IMPROVEMENT IN FAGOTS OR PILES FOR MANUFACTURING RAILROAD-RAILS.

Specification forming part of Letters Patent No. **79,904**, dated July 14, 1868.

*To all whom it may concern:*

Be it known that we, WILLIAM HAYWARD and JOHN LEES, of Danville, in the county of Montour and State of Pennsylvania, have invented a new and useful Improvement in Manufacturing Rails; and we do hereby declare that the following is a full, clear, and exact description thereof, which will enable those skilled in the art to make and use the same, reference being had to the accompanying drawings, forming part of this specification.

This invention relates to the manufacture of rails for railroads of iron or steel, or iron and steel combined; and it consists in forming what is known as a "pile" for rolling in the manner hereinafter described.

In the drawings Figure 1 represents a longitudinal section of the pile; and Fig. 2 is an end view of the same, showing the shape of the parts which form the pile.

Similar letters of reference indicate corresponding parts.

In rolling out railroad-rails a pile is formed of two or more separate pieces of iron or steel, (or iron and steel combined, if the rail is to have a steel wearing-surface,) and the same is subjected to a high temperature in the furnace and passed through the rollers and formed into rails of any required shape, the parts being firmly welded together by the rolling process. Different qualities of iron are combined in this manner, or iron and steel, so that a supe-

rior quality of iron or steel may form the face or wearing-surface of the rail, while the less important part is formed of an inferior quality of metal.

In carrying out our invention we form the pile as seen in Fig. 2.

A, B, and C are three differently-shaped bars of iron, which are rolled to fit together, substantially as seen.

By placing the bars together, as seen in the drawings, the pile may be made as high as may be desired, while each separate piece will be held to its place by the pieces with which it is combined.

The pieces or bars A may be dispensed with, and only the pieces or bars B and C be retained, if desired.

By making the pile in this manner the operation of rolling or manufacturing rails of the various kinds is greatly facilitated, while a much superior rail is produced, as compared with the ordinary method of piling.

We claim as new and desire to secure by Letters Patent—

The pile as represented in the drawings, either with or without the part A, substantially as shown, as and for the purposes set forth.

WILLIAM HAYWARD.  
JOHN LEES.

Witnesses:

PETER BALDY, Jr.,  
H. W. HUNTER.